

## UNITED STATES PATENT OFFICE.

ALFRED BREWERTON CRAVEN, OF SELBY, ENGLAND, ASSIGNOR, BY MESNE ASSIGNMENTS, TO YORKSHIRE DYEWARE & CHEMICAL COMPANY LIMITED, OF LEEDS, YORK, ENGLAND.

## MANUFACTURE OF LINOLEUM AND THE LIKE.

No Drawing.

Application filed October 31, 1918. Serial No. 260,585.

*To all whom it may concern:*

Be it known that I, ALFRED BREWERTON CRAVEN, subject of the King of Great Britain, residing at Selby, Yorkshire, in the 5 Kingdom of England, have invented certain new and useful Improvements in and Relating to the Manufacture of Linoleum and the like, of which the following is a specification.

10 The present invention relates to improvements in the manufacture of linoleum consisting in the use of a new material for this purpose and the invention is also designed to utilize more effectively certain by-products obtained in the oil manufacturing industry.

15 The by-products I employ are those consisting of liquid or semi-solid mixtures of fatty acids and glycerides in varying proportions and mucilage and colouring matter 20 obtained in refining for edible and other purposes drying and/or partially drying oils. The refining operations which yield the by-products I use are those generally in use and 25 consists of, for example: (a) Treatment of crude oil with a small quantity of strong soda lye sufficient to combine with the free fatty acids present and to leave a slight excess of caustic soda, agitating well and warming gently then allowing to stand, 30 when the soap formed settles to the bottom carrying down with it colouring matter mucilage and some of the oil itself. The clear refined oil is run off and leaves the foots as by-product which I acidify with 35 mineral acid to convert the soap into fatty acids, and wash to remove mineral acid and its salt. (b) Refining by acid treatment which consists of heating and agitating the crude oil with a small amount of slightly diluted sulphuric acid and allowing to stand. 40 When the clear oil is run off, the sediment consisting of mucilage and oil is a suitable by-product after being washed free from mineral acid. (c) Similar sediments resulting from other processes of refining such as 45 treatment with bichromate of potash and mineral acid, and any sediment formed when a partly refined drying or partially drying oil, or boiled oil is allowed to stand in a tank, are all suitable for my process. (d)

50 The oily matter absorbed by fuller's earth which has been used in refining is also suitable when extracted from the fuller's earth by a volatile solvent or by other means.

I could use the commercial drying oils and/ or partly drying oils, or mixtures of these oils and their fatty acids, or their commercial fatty acids, but I prefer to make use of the by-products above mentioned as the most economical source of my raw materials. 55

The new material I use for the manufacture of linoleum is the resilient tacky and adhesive residue obtained from the distillation of the aforesaid by-products. The foots and waste products from the oil manufacturing industry are usually worked up by distillation and the main object is to obtain commercially usable fatty acids as a distillate. The residue left in the still at the end of this operation usually consists of black 60 pitch which is of low commercial value.

This by-product of distillation (the residue) is usually quite unsuitable for use in the manufacture of linoleum. I have found, however, that whereas the foots from non-drying oils and fats on distillation yield dark non-resilient and brittle residues which are unsuitable for linoleum manufacture that on the contrary those from drying oils and/or partially drying oils, or mixtures 70 largely consisting thereof, can be distilled in such manner as to yield a product which is very valuable for use in making a cement for linoleum manufacture. According to the 75 present invention I keep separate the waste products so that they contain only those from the drying oils or partially drying oils and are free from the products of non-drying oils and I distil them with the definite object of obtaining a product which will be 80 useful in linoleum manufacture. The oils which are suitable for my purpose and which are sources of the materials I distil to obtain the residue I use are, linseed oil, cotton seed oil, soya bean oil, whale oil, menhaden oil, cod oil, and other oils which contain 85 fatty acids or glycerides capable of polymerization under the conditions of working.

The distillation is to be conducted in such manner and stopped at such a stage that a 90 large yield is obtained of a residue which is resilient, adhesive and showing maximum paleness of colour and freedom from smell, by virtue of which qualities the product becomes suitable for linoleum manufacture. 95

The by-products from drying oils may be 100 distilled without mixture with by-products from partly-drying oils, or the latter by-

products may be distilled without mixture with drying oil by-products, or the by-products from drying oils and partly-drying oils may be mixed and distilled together, but I do not mix any by-products of non-drying oils with those of the other classes but ensure the absence of non-drying oil by-products by having them kept separate in the works where they are made. The distillation of by-products from drying and partly-drying oils without any non-drying oil by-products yields a distillate of fatty acids of at least as high commercial value as is obtained when the by-products from all the classes of oils are mixed indiscriminately and distilled, which is the usual commercial practice.

The temperature and mode of distillation are to be regulated so as to secure the above mentioned properties in the residue, but I have further found that an increased yield of residue of the desired properties can be obtained from the waste oil products of both drying oils and partially drying oils by thickening the oil by-products and this thickening may be effected by heating before the distillation commences.

The distillation process removes from the fatty matter certain solid saturated fatty bodies which are detrimental for my purpose, i. e., myristic, palmitic and stearic acids and also the fluid unsaturated oleic acid which is also detrimental. The more unsaturated acids (linolic, elupanodonic and linolenic) and their glycerides become thickened or polymerized. The heat is supplied by a fire under the still and the temperature may reach 300 degrees C., and the heat is maintained until a decided thickening, due to polymerization of the more unsaturated bodies has taken place. During distillation, thickening also takes place, due to polymerization, and also due to the removal of non-thickening bodies, and leaves behind, when stopped at the right stage, the resiliant, tacky and adhesive mass.

The paleness and freedom from smell are improved by rigid exclusion of air during thickening and during distillation, e. g.; by working in an airtight still in vacuo, or in presence of an inert gas, e. g., carbon dioxide or by superheated steam or by a combination of these methods. The waste fatty products may be treated by any known method in order to remove foreign matter and fat and improve the colour before submission to the thickening and distillation.

The colour of the by-products may be improved or bleached by heating with a solution of bleaching powder and then adding mineral acid and washing free from mineral acid. Or by washing with strong alkaline lye, which dissolves the colour and also forms soap which is almost insoluble in the strong lye. The coloured lye is run away from the soap and the soap decomposed with

mineral acid and the paler oil product is washed.

The filtration of the by-products may be done in a filter press when the by-products are pumped in and a pressure maintained to hasten the operation and to yield a cake of fatty matter and foreign matter of some firmness which may be further pressed in a hydraulic press to yield more clear oil products. The clear portion from both these operations is distilled. The removal of the solid fat reduces the time required for the production of the residue, because the bodies which produce the particular residue I make, are liquid at ordinary temperatures, and any solid fat introduced into the still must be removed by the distillation before the residue can have the required characteristics. Other known methods of bleaching and removal of solid bodies may be used with the same object.

#### Example.

The foots from any drying oils or partly drying oils, (but not non-drying oils) such as tank bottoms, or the sediment from refining the above oils in the manner described above, are treated to remove the colouring matter, by washing with strong alkaline lye or other suitable means, and decomposing the soap with mineral acid and washing free from mineral acid. Thirty cwts. of the product are charged into a still made of cast iron provided with a safety valve and arranged to be heated by fire. The air is exhausted and then the still is closed airtight. The fire is started and the temperature raised to 270 to 300 degrees C., and maintained thereat for 1 to 2 hours, any undue pressure developed during this heating is relieved by the safety valve, and then the outlet for the distillate is opened and superheated steam passed through the fatty matter in the still and the temperature is regulated to give a steady delivery of pale fatty acid distillate and water. This distilling is continued until the residue left in the still is non-greasy and when cold, resiliant, tacky and adhesive. This residue is then run out, and may be used for the manufacture of linoleum and the like.

The product may be used in the usual way by incorporating it with cork or wood fibre and pigments so as to form linoleum, or it may be used in conjunction with linoleum cement made from linseed oil or the like for the manufacture of linoleum or other material. The product itself may also be used for the other known purposes for which linoleum cement made from linseed oil is suitable. During or after the manufacture of the product gum resin, or other bodies may be added to the product to make it more suitable for purposes of linoleum manufacture.

I declare that what I claim is:—

1. The process of obtaining an agglutinant for the manufacture of linoleum which consists in submitting to a distilling 5 temperature, out of contact with free oxygen substances containing the radical of an unsaturated acid more unsaturated than oleic acid, and of the kind occurring in more or less drying oils, until the residue goes beyond the varnish stage and becomes semi-solid, resilient, tacky and adhesive:—the agglutinant aforesaid.
2. The process of obtaining an agglutinant for the manufacture of linoleum consisting 15 of submitting oils of a more or less drying character to a distilling temperature out of contact with free oxygen when the non-drying portion of the oils distils over and the residue goes beyond the varnish stage and 20 becomes semi-solid resilient tacky and adhesive—the agglutinant aforesaid.
3. The process of obtaining an agglutinant for the manufacture of linoleum consisting of submitting a mixture of more or less drying 25 oils and their fatty acids to a distilling temperature out of contact with free oxygen when the non-drying portion of the mixture distils over and the residue goes beyond the varnish stage and becomes semi-solid 30 silent, tacky and adhesive.
4. The process of obtaining an agglutinant for the manufacture of linoleum consisting of submitting fatty acids from more or less drying oils to a distilling temperature 35 out of contact with free oxygen when the non-drying portion of the fatty acids distils over and the residue goes beyond the varnish stage and becomes semi-solid, 40 resilient, tacky and adhesive.
5. The process of obtaining an agglutinant from the purification residues of more or less drying oils for the manufacture of linoleum consisting of submitting 45 such by-products without admixture of by-products from non-drying oils or fats to a distilling temperature out of contact with free oxygen when the non-drying portion of these by-products distils over and the residue goes beyond the varnish stage and 50 becomes semi-solid, resilient, tacky, and adhesive.
6. The process of obtaining an agglutinant for the manufacture of linoleum consisting of distilling substances containing the radical of a fatty acid more unsaturated than oleic acid in a current of superheated steam to assist in the removal of non-drying matter therefrom from any of the materials mentioned in claim 1. 55
7. The process of obtaining an agglutinant 60 for linoleum containing the purification residue from by-products from more or less drying oils which consists of submitting the said by-products to a preliminary filtration and then submitting them to a distilling 65 temperature out of contact with free oxygen.
8. That step in the process of obtaining an agglutinant for linoleum from the materials as set forth in claim 1, which consists in bleaching the said materials before 70 the distillation operation, with the object of producing a paler agglutinant.
9. The process of obtaining an agglutinant for linoleum from the materials mentioned in claim 1, which consists in first 75 submitting the said materials to a preliminary heating for a prolonged period as described out of contact with free oxygen whereby the oil is polymerized and then submitting the materials to a distilling temperature 80 out of contact with free oxygen.
10. As a new article of manufacture a semi-solid tacky and adhesive distillation residue for mixing with powdered cork and the like, for making linoleum which consists 85 of the bodies mentioned in claim 1 thickened and more or less polymerized beyond the varnish stage, such material being of a tacky and adhesive character and semi-solid at ordinary room temperature but substantially 90 free from non-drying oil derivatives and consisting substantially of polymerized bodies derived from acids more unsaturated than oleic acid. 95

In witness whereof, I have hereunto signed my name this 8th day of October 1918, in the presence of two subscribing witnesses.

ALFRED BREWERTON CRAVEN.

Witnesses:

LUCY COSTIGAN,  
R. RAYMOND HAYNES.